# EUROPEAN PATENT SPECIFICATION

(11) **EP 0 385 633 B1**
(45) Date of publication and mention of the grant of the patent: **07.04.1993**
(21) Application number: 90301791.1
(22) Date of filing: 20.02.1990
(51) Int. Cl.: C10L 1/22, C10L 1/14

(54) **Middle distillate fuel having improved storage stability**
Lagerungsbeständiger Mitteldestillatkraftstoff
Combustible de distillat moyen ayant une stabilité au stockage modifiée

(30) Priority: 02.03.1989 US 318748
(43) Date of publication of application: 05.09.1990
(62) Divisional of application: 90116830.2
(73) Proprietor: ETHYL PETROLEUM ADDITIVES, INC., St. Louis Missouri 63102-1886 (US)
(72) Inventor: Bostick, John Gray, Smithtown Illinois 62285 (US); Cunningham, Larry John, Kirkwood Missouri 63122 (US); Hanlon, John Vincent, St.Louis, Missouri 63131 (US)
(74) Representative: Collier, Jeremy Austin Grey

(56) References cited:
- EP-A- 0 182 940
- EP-A- 0 261 795
- EP-A- 0 294 045
- US-A- 2 928 790
- US-A- 3 442 791
- US-A- 3 701 641
- US-A- 4 025 316
- US-A- 4 166 726
- US-A- 4 172 707

## Description

This invention relates generally to improving the stability of middle distillate fuels and more particularly to stabilized middle distillate fuel compositions which contain a combination of N,N-dimethylcyclohexyl amine and a Mannich Base.

Middle distillate fuels such as diesel oil, fuel oil, jet fuel and kerosene when stored for long periods of time are subject to the formation of color and solid deposits. The deposits accumulate on filters causing the filters to become plugged. Various additives and combinations of additives have been employed to reduce color and deposit formation. For example: U.S. Patent 2,984,550 discloses the use of Mannich bases derived from phenols, formaldehyde and polyamines for stabilization; U.S. Patent 3,490,882 discloses stabilized petroleum distillate fuel oils containing N,N-dimethylcyclohexylamine antioxidant and a N,N′-di(ortho-hydroxyarylidene)-1,2-alkylenediamine metal deactivator such as N,N′-disalicylidene-1,2-propylenediamine; U.S. Patent 4,166,726 discloses a fuel additive which is a mixture of a polyalkylene amine and a Mannich Base; and U.S. Patents 4,501,595 and 4,533,361 disclose diesel oil which contains a condensate of tetraethylene pentamine, paraformaldehyde, a hindered phenol such as 2,6-di-t-butylphenol and polyisobutenyl succinic anhydride.

The effectiveness of any particular type of additive combination can vary with different fuel stocks and combinations which are more effective at the same total additive concentration reduce treatment cost. We have now discovered novel, synergistic additive combinations which include certain Mannich Bases and provide middle distillate fuels having generally improved storage stability compared to fuels containing the same total concentrations of either N,N-dimethylcyclohexylamine antioxidant alone or N,N-dimethylcyclohexylamine in combination with an N,N′-di(ortho-hydroxyarylidene)-1,2-alkylenediamine metal deactivator.

In accordance with this invention, there is provided a fuel additive concentrate comprising a mixture of N,N-dimethylcyclohexylamine and a Mannich Base which is the reaction product of an aldehyde, an amine and an alkyl phenol selected from (a) hindered phenol having the formula:
where R₁, R₂, R₃ are independently selected from hydrogen, t-butyl, t-amyl and isopropyl, provided that at least one of R₁, R₂ and R₃ is hydrogen and at least one of R₁ and R₂ is t-butyl, t-amyl or isopropyl; and (b) p-alkyl phenol having the formula:
where R₄ is C₉ to C₃₀ alkyl.
The concentrate can also contain a N,N′-di(ortho-hydroxyarylidene)-1,2-alkylenediamine metal deactivator such as N,N′-disalicylidene-1,2-propylenediamine. Also provided is a stabilized fuel containing from 1 to 1400 mg/l of N,N-dimethylcyclohexylamine, from 0.5 to 1100 mg/l of Mannich Base and from 0 to 400 mg/l of an N,N′-di(ortho-hydroxyarylidene)-1,2-alkylenediamine.

The N,N-dimethylcyclohexylamine component of the compositions of the invention is a commercially available fuel antioxidant.

The N,N′-di(ortho-hydroxyarylidene)-1,2-alkylenediamine component, in which, typically, the arylidene radical contains 6-7 carbon atoms and the alkylene radical contains 2-3 carbon atoms, is a metal deactivator whose presence in combination with the other components provides fuel compositions of the invention having the most improved stability. The preferred metal deactivator is N,N′-disalicylidene-1,2-propylenediamine which is commercially available.

The Mannich Base component of the invention is produced by the Mannich condensation reaction of a hindered or p-alkyl phenol, an aldehyde, such as formaldehyde, ethanal, propanal, and butanal (preferably formaldehyde in its monomeric form or paraformaldehyde) and primary and secondary amines.

The hindered phenols which are useful in preparing the Mannich Base component of the invention are phenols which are characterized by the presence of at least one and preferably two ortho-t-butyl, t-amyl, and/or isopropyl groups. Specific examples of such hindered phenols include: 2,4-di-t-butylphenol, 2,4-diisopropylphenol, 2,6-diisopropylphenol, 2-t-butylphenol, and 2-t-amylphenol with 2,6-di-t-butylphenol being most preferred.

The p-alkyl phenols which are useful in preparing the Mannich Base component of the invention are those which contain from 9 to 30 carbons which can be arranged in either a straight or a branched chain. Preferred phenols are C₉ to C₁₂ p-alkylphenols such as, for example, p-nonylphenol and p-dodecylphenol.

The amines which are useful in preparing the Mannich Base component of the invention are primary and secondary amines which can be selected from one or more of:
A. alkyl monoamines of the formula; where R₅ is selected from H and C₁ to C₅ alkyl, and R₆ is selected from C₁ to C₁₄ alkyl and the group -(CH₂)n-OR₇ where n = 1 to 10 and R₇ is C₁ to C₂₀ alkyl,
B. alkyl diamines of the formula; where R₅ is selected from H and C₁ to C₅ alkyl, R₈ is C₁ to C₆ alkylene and A and B are independently selected from H, C₁ to C₅ alkyl, mono-hydroxysubstituted C₁ to C₅ alkyl, and the group (CH₂)ₙ-OR₇ where n = 1 to 10 and R₇ is C₁ to C₂₀ alkyl,
C. ethylene polyamines of the formula;
   ${\text{H₂N(̵(CH₂)₂NH)̵}}_{\text{n}} \text{H}$ where n = 2 to 10, and
D. cyclic amines of the formula; where n and m are independently integers from 1 to 3, X is selected from CH₂, O, S and NR₉ where R₉ is H, C₁ to C₁₀ alkyl, or the group (CH₂)ₙ-NH₂ where n is 1 to 10. The alkyl groups can have a branched chain.

Specific examples of such amines include 1,3-diaminopropane, 1,2 diaminopropane, dimethylamine, diethylamine, dipropylamine, dibutylamine, N,N-dimethyl-1,3-diaminopropane, 1,1-dimethyldodecylamine, mixed C₁₂-C₁₄ t-alkyl amines, 2-methyl-1,5-pentadiamine, ethylenediamine; cyclic amines such as piperazine, aminoethylpiperazine, morpholine and thiomorpholine; and ethylene polyamines such as diethylene triamine and triethylene tetraamine.

The Mannich Base can be formed by reacting from 1 to 5 moles of aldehyde, from about 1 to 2 moles of amine and from 1 to 4 moles of phenol at a temperature of from 0°C to 150°C for 0.5 to 10 hours. An inert solvent such as isopropanol can be used which is distilled from the product along with water formed in the reaction.

The Mannich Base product is usually a mixture of materials which may contain unreacted ingredients, especially the phenol. The Mannich Bases can be isolated from the product mixture but the product mixture itself can conveniently be used in forming the compositions of the invention. Examples of Mannich reactions and products are illustrated below:
or
where R₁, R₂, R₄, R₅ and R₆ are as defined above.

The additive mixtures of the invention are usually prepared and marketed in the form of concentrates for addition to the fuel by the customer although the individual components could be added directly into the fuel. Suitable proportions of additives in the concentrates of the invention, based on the total weight of concentrate, include from 25 to 95 wt% N,N-dimethylcyclohexylamine, from 0 to 25 wt% N,N′-di(ortho-hydroxyarylidene)-1,2-alkylenediamine and, from 5 to 75 wt% Mannich Base.

The concentrates are added to the fuel in effective amounts to provide improved stability. Suitable amounts of additive concentrate in the fuel are from 1 to 500 pounds per thousand barrels (Ptbs) (3 to 1500 mg/l, preferred 2.5 to 100 Ptbs or 8 to 300 mg/l). This will provide a stabilized fuel containing from 1 to 1400 mg/liter (preferred 2 to 250 mg/l) N,N-dimethylcyclohexylamine, from 0 to 400 mg/l (preferred 0 to 100 mg/l) N,N′-di(ortho-hydroxyarylidene)-1,2-alkylenediamine metal deactivator and from 1 to 1100 mg/l (preferred 1 to 250 mg/l) of Mannich Base. When used, the metal deactivator is present in amounts of 1.0% to 25 wt% of concentrate or .3 to 400 mg/l of fuel. The concentrates can also contain an inert diluent or solvent which can be, for example, an aliphatic hydrocarbon such as kerosene or an aromatic hydrocarbon such as xylene.

The middle distillate fuels whose stability is improved by the invention typically include those boiling within a temperature range of 150°-400°C which may commonly be labeled as kerosene, fuel oil, diesel oil, No. 1-D, or No. 2-D.

The compositions of the invention are further illustrated by, but are not intended to be limited to, the following examples wherein parts are parts by weight unless otherwise indicated.

### Example 1

A Mannich Base reaction product of formaldehyde, 1,3-diaminopropane and 2,6-di-t-butylphenol is prepared by the following process.

Dissolve 103 grams (0.5 mole) of 2,6-di-t-butylphenol in 100 grams of isopropyl alcohol (IPA) in a 500 ml round bottom flask. Add 18.5 grams (0.25 mole) of 1,3-diaminopropane dropwise over 15 minutes while the contents of the flask are stirred. There is an exotherm observed as the amine is added. Cool the contents of the flask to below 30°C and add a 10% excess, (44.6 grams 0.55 mole) of 37% aqueous formaldehyde solution dropwise over 30 minutes while maintaining the temperature below 30°C. Heat the contents of the flask to reflux and continue to reflux for one hour. Switch from reflux to distillation and distill off IPA/water mixture to 105°C. Apply 28 in. Hg vacuum to remove residual materials. The total product yield is 122.2 or 96% of theory which contains compounds of the Structure III and IV.

Additive blends of the reaction product were prepared and tested in different fuels using both the D 4625 43°C (110°F) Storage Stability Test, in which the color change (using ASTM D1500) and the total insolubles in the fuel (reported in mg/100 ml) are determined on 400 ml samples stored for 13 weeks in the dark and the F-21-61 149°C (300°F) Accelerated Stability Test in which the color change and insoluble gums are determined on 50 ml samples heated to 149°C for a selected time, which was 90 minutes, allowed to cool in the dark, tested for color (ASTM D1500), and then filtered (using a 4.25 cm Whatman #1 filter paper) and the filtrate discarded. The filter is washed clean of fuel with isooctane and measured for deposits by comparison with a set of reference papers. The blend compositions and test results in comparison to untreated fuel and blends without the Mannich Base product are reported in Table I below.

A significant difference in stability at 149°C is indicated by a color difference of about 1/2 number and/or a deposit difference of 2 numbers and a significant difference in stability at 43°C is indicated by a color difference of about 1/2 number and a deposit difference of 20%. The results in Table I show that the blends of the invention which contain Mannich Base in addition to DMCA or DMCA and MDA gave significantly better overall stability when compared to comparable blends which did not contain the Mannich Base, for example, blend 3 vs blend 2 and blend 5 vs blend 4 of Fuel #1.

### Example 2

A Mannich Base reaction product of formaldehyde, dimethylamine, and 2,6-di-t-butylphenol is prepared by the following process.

Dissolve 103 grams (0.5 mole) of 2,6-di-t-butylphenol in 100 grams of IPA in a 500 ml round bottom flask and add 72 grams (0.64 mole) of a 40% aqueous dimethylamine solution. Cool the mixture to about 30°C and add dropwise with stirring 44.6 grams (0.55 mole) of 37% formaldehyde while keeping the mixture at a temperature below 40°C. Heat the mixture to reflux and reflux for 4 hours. Remove IPA/water by distillation and apply vacuum to remove residual materials. The product yield is 113 grams or 86% of theory which contains N,N-dimethyl-3,5-di-t-butyl4-hydroxybenzylamine.

Additive blends of the above reaction product were prepared and tested in different fuels using the test procedures described in Example 1. The blend compositions and test results in comparison to untreated fuel and blends which did not contain the Mannich Base product are reported in Table II below.

The results indicated that the blends containing Mannich Base gave fuels having significantly improved stability except in the case of Fuel #4 where the results were mixed.

### Example 3

A Mannich Base reaction product of formaldehyde, C₁₂-C₁₄ t-alkyl amine mixture (Primene 81R) and 2,6-di-t-butyl phenol is prepared by the process described in Example 2 using 95.5 grams (0.5 mole) of Primene 81R in place of the dimethylamine. The product yield is 200 grams or 82% of theory which contains N-[3,5-di-t-butyl-4-hydroxybenzyl]-mixed C₁₂-C₁₄ t-alkyl amines.

Additive blends of the above reaction product were prepared and tested in #2 diesel fuel using the test procedures described in Example 1. The blend compositions and test results are reported in Table III below.

The results indicate that blends 4 and 7 according to the invention which contain the Mannich Base in addition to DMCA and MDA have better stability at the same total additive levels compared to blends 2 and 5 containing only DMCA and MDA.

### Example 4

A Mannich Base reaction product of formaldehyde, 1,2-diaminopropane, and 2,6-di-t-butyl phenol is prepared by the following process.

Dissolve 103 gm (0.5 mole) of 2,6-di-t-butyl phenol in 100 grams of IPA in a 500 ml roundbottom flask and add 18.5 grams (0.25) moles of 1,2-diaminopropane. Cool this mixture to about 30°C and add dropwise with stirring 44.6 grams (0.55 mole) of 37% formaldehyde while keeping the temperature of the mixture below 40°C. Heat the mixture to reflux and reflux for 1 hour. Remove IPA/water by distillation and apply vacuum to remove residual materials.

Additive blends of the above reaction product were prepared and tested in Fuel #1 fuel using the test procedures described in Example 1. The blend compositions and results are reported in Table IV below.

The results indicate that blend 4 of the invention containing the Mannich Base has improved stability compound to blend 2 which containing DMCA alone. Blend 5 containing the Mannich Base has improved stability over blend 3 which contained DMCA and MDA alone.

### Example 5

A Mannich Base reaction product of formaldehyde, N,N-dimethyl-1,3-diaminopropane, and p-dodecylphenol was prepared by the following procedure.

Combine 262.4 grams (1.0 mole) of the alkyl (C₁₂) phenol with 102.2 grams (1.0 mole) of N,N-dimethyl-1,3-diamino-propane and add 89.2 grams (1.1 mole) of 37% formaldehyde with stirring while keeping the temperature below 40°C. Heat the mixture to 100°C for two hours and then remove water by distillation (100°C - 28 in vacuum). The product yield is 176 grams or 93% of theory which contains N,N-dimethyl-N′-[2 hydroxy-5-dodecylbenzyl]-1,3-diaminopropane.

Additive blends of the above reaction product were prepared and tested in midcontinent #2 diesel fuel using the test procedures described in Example 1. The blend compositions and results are reported on Table V below.

The results indicate that blends 3 and 5 of the invention have over-all improved stability compared to blends at the same total additive level which did not include the Mannich Base.

## Claims

1. A fuel additive concentrate comprising a mixture of N,N-dimethylcyclohexylamine and a Mannich Base which is the reaction product of an aldehyde, a primary or secondary amine and an alkyl phenol selected from (a) hindered phenol having the formula: where R₁, R₂, R₃ are independently selected from hydrogen, t-butyl, t-amyl and isopropyl, provided that at least one of R₁, R₂ and R₃ is hydrogen and at least one of R₁ and R₂ is t-butyl, t-amyl or isopropyl; and (b) p-alkyl phenol having the formula: where R₄ is C₉ to C₃₀ alkyl; said concentrate containing, based on the total weight of concentrate, from 25 to 95 wt% N,N-dimethylcyclohexylamine from 5 to 75 wt% Mannich Base.

2. The concentrate of claim 1 wherein the concentrate also contains from 1 to 25 wt% N,N′-di(ortho-hydroxyarylidene)-1,2-alkylenediamine metal deactivator.

3. The concentrate of claim 1 or 2 wherein the aldehyde is formaldehyde, and the amine is selected from one or more of:
A. alkyl monoamines of the formula; where R₅ is selected from H and C₁ to C₅ alkyl, and R₆ is selected from C₁ to C₁₄ alkyl and the group -(CH₂)n-OR₇ where n = 1 to 10 and R₇ is C₁ to C₂₀ alkyl,
B. alkyl diamines of the formula; where R₅ is selected from H and C₁ to C₅ alkyl, R₈ is C₁ to C₆ alkylene and A and B are independently selected from H, C₁ to C₅ alkyl, mono-hydroxysubstituted C₁ to C₅ alkyl, and the group (CH₂)ₙ-OR₇ where n = 1 to 10 and R₇ is C₁ to C₂₀ alkyl,
C. ethylene polyamines of the formula;
${\text{H₂N(̵(CH₂)₂NH)̵}}_{\text{n}} \text{H}$ where n = 2 to 10, and
D. cyclic amines of the formula; where n and m are independently intergers from 1 to 3, X is selected from CH₂, 0, S and NR₉ where R₉ is H, C₁ to C₁₀ alkyl, or the group (CH₂)ₙ-NH₂ where n is 1 to 10.

4. The concentrate of any of the preceding claims wherein the phenol is a hindered phenol, and the Mannich Base comprises N-[3,5-di-t-butyl-4-hydroxybenzyl]-mixed C₁₂ to C₁₄ t-alkyl amines, N,N-dimethyl-3,5-di-t-butyl-4-hydroxybenzylamine, a compound of the formula: where R₁ and R₂ are independently selected from hydrogen, t-butyl, t-amyl and isopropyl provided that at least one of R₁ and R₂ is t-butyl, t-amyl, or isopropyl, or a compound of the formula: where R₁ and R₂ are independently selected from hydrogen, t-butyl, t-amyl and isopropyl provided that at least one of R₁ and R₂ is t-butyl, t-amyl, or isopropyl.

5. The concentrate of any of claims 1-3 wherein the phenol is a p-alkylphenol, and the Mannich Base comprises N,N-dimethyl-N′-[2-hydroxy-5-dodecylbenzyl]-1,3-diaminopropane.

6. The concentrate of claim 2 wherein the metal deactivator is N,N′-disalicylidene-1,2-propylenediamine and the Mannich Base is the reaction product of formaldehyde, 2,6-di-t-butyl phenol and an amine selected from 1,3-diaminopropane, 1,2-diaminopropane, mixed C₁₂-C₁₄ t-alkyl amines, and dimethylamine.

7. The concentrate of claim 2 wherein the metal deactivator is N,N′-disalicylidene-1,2-propylenediamine and the Mannich Base is the reaction product of formaldehyde, p-dodecyl phenol, and N,N-dimethyl-1,3-diaminopropane.

8. A fuel composition comprising middle distillate fuel containing from 3 to 1500 mg/l of the concentrate of any of claims 1-7.

9. A fuel composition comprising a middle distillate fuel and from 1 to 1400 mg/l N,N-dimethylcyclohexylamine, from 0 to 400 mg/l N,N-di(ortho-hydroxyarylidene)-1,2-alkylenediamine and from 1 to 1100 mg/l of a Mannich Base which is the reaction product of an aldehyde, an amine and an alkyl phenol selected from (a) hindered phenol having the formula: where R₁, R₂, R₃ are independently selected from hydrogen, t-butyl, t-amyl and isopropropyl, provided that at least one of R₁, R₂ and R₃ is hydrogen and at least one of R₁ and R₂ is t-butyl, t-amyl or isopropyl; and (b) p-alkyl phenol having the formula: where R₄ is C₉ to C₃₀ alkyl.

10. The fuel composition of claim 9 wherein the aldehyde is formaldehyde and the amine is selected from one or more of:
A. alkyl monoamines of the formula; where R₅ is selected from H and C₁ to C₅ alkyl and R₆ is selected from C₁ to C₁₄ alkyl and the group -(CH₂)n-OR₇ where n = 1 to 10 and R₇ is C₁ to C₂₀ alkyl,
B. alkyl diamines of the formula; where R₅ is selected from H and C₁ to C₅ alkyl R₈ is C₁ to C₆ alkylene and A and B are independently selected from H, C₁ to C₅ alkyl, monohydroxysubstituted C₁ to C₅ alkyl, and the group (CH₂)ₙ-OR₇ where n = 1 to 10 and R₇ is C₁ to C₂₀ alkyl,
C. ethylene polyamines of the formula;
${\text{H₂N(̵(CH₂)₂NH)̵}}_{\text{n}} \text{H}$ where n = 2 to 10, and
D. cyclic amines of the formula; where n and m are independently intergers from 1 to 3, X is selected from CH₂, O, S and NR₉ where R₉ is H, C₁ to C₁₀ alkyl, or the group (CH₂)ₙ-NH₂ where n is 1 to 10.

## Patentansprüche

1. Treibstoffzusatzkonzentrat umfassend eine Mischung aus N,N-Dimethylcyclohexylamin und einer Mannich-Base, die das Reaktionsprodukt eines Aldehyds, eines primären oder sekundären Amins und eines Alkylphenols ist, das ausgewählt ist aus (a) gehindertem Phenol mit der Formel in der R₁, R₂ und R₃ unabhängig voneinander aus Wasserstoff, t-Butyl, t-Amyl und Isopropyl ausgewählt sind, mit der Maßgabe, daß mindestens einer der Reste R₁, R₂ und R₃ Wasserstoff ist und mindestens einer der Reste R₁ und R₂ t-Butyl, t-Amyl oder Isopropyl ist, und
(b) p-Alkylphenol mit der Formel in der R₄ C₉-C₃₀-Alkyl ist, wobei das Konzentrat auf der Basis seines Gesamtgewichts zwischen 25 und 95 Gew.-% N,N-Dimethylcyclohexylamin und 5 bis 75 Gew.-% Mannich-Base enthält.

2. Konzentrat nach Anspruch 1, welches außerdem zwischen 1 und 25 Gew.-% N,N′-Di(ortho-hydroxyaryliden)-1,2-alkylendiamin-Metalldeaktivator enthält.

3. Konzentrat nach Anspruch 1 oder 2, in dem das Aldehyd Formaldehyd ist und das Amin ausgewählt ist aus einer oder mehreren der folgenden Substanzen:
A. Alkylmonoamine der Formel in der R₅ ausgewählt ist aus H und C₁- bis C₅-Alkyl und R₆ ausgewählt ist aus C₁- bis C₁₄-Alkyl und der Gruppe -(CH₂)n-OR₇, in der n = 1 bis 10 ist und R₇ C₁-C₂₀-Alkyl ist,
B. Alkyldiamine der Formel in der R₅ ausgewählt ist aus H und C₁- bis C₅-Alkyl, R₈ C₁- bis C₆-Alkylen ist und A und B unabhängig voneinander aus H, C₁- bis C₅-Alkyl, mono-hydroxysubstituiertem C₁- bis C₅-Alkyl und der Gruppe (CH₂)ₙ-OR₇, in der n = 1 bis 10 ist und R₇ C₁- bis C₂₀-Alkyl ist, ausgewählt sind.
C. Ethylenpolyamine der Formel
H₂N(̵(CH₂)₂NH)̵ₙH, in der n = 2 bis 10 ist, und
D. cyclische Amine der Formel in der n und m unabhängig ganze Zahlen von 1 bis 3 sind, X ausgewählt ist aus CH₂, 0, S und NR₉, worin R₉ H, C₁- bis C₁₀-Alkyl oder die Gruppe (CH₂)ₙ-NH₂ ist, in der n 1 bis 10 beträgt.

4. Konzentrat nach einem der vorstehenden Ansprüche, in dem das Phenol ein gehindertes Phenol ist und die Mannich-Base N-[3,5-di-t-Butyl-4-hydroxybenzyl]-vermischte C₁₂- bis C₁₄-t-Alkylamine, N,N-Dimethyl-3,5-di-t-butyl-4-hydroxybenzylamin, eine Verbindung der Formel: in der R₁ und R₂ unabhängig voneinander aus Wasserstoff, t-Butyl, t-Amyl und Isopropyl ausgewählt sind, mit der Maßgabe, daß mindestens einer der Reste R₁ und R₂ t-Butyl, t-Amyl oder Isopropyl ist, oder eine Verbindung der Formel in der R₁ und R₂ unabhängig aus Wasserstoff, t-Butyl, t-Amyl und Isopropyl ausgewählt sind, mit der Maßgabe, daß mindestens einer der Reste R₁ und R₂ t-Butyl, t-Amyl oder Isopropyl ist, umfaßt.

5. Konzentrat nach einem der Ansprüche 1 bis 3, in dem das Phenol ein p-Alkylphenol ist und die Mannich-Base N,N-Dimethyl-N′-[2-hydroxy-5-dodecylbenzyl]-1,3-diaminopropan enthält.

6. Konzentrat nach Anspruch 2, in dem der Metalldeaktivator N,N′-Disalicyliden-1,2-propylendiamin und die Mannich-Base das Reaktionsprodukt aus Formaldehyd, 2,6-Di-t-butylphenol und einem aus der Gruppe 1,3-Diaminopronan, 1,2-Diaminopropan, gemischten C₁₂-C₁₄-t-Alkylaminen und Dimethylamin ausgewählten Amin ist.

7. Konzentrat nach Anspruch 2, in dem der Metalldeaktivator N,N′Disalicyliden-1,2-propylendiamin und die Mannich-Base das Reaktionsprodukt aus Formaldehyd, p-Dodecylphenol und N,N-Dimethyl-1,3-diaminopropan ist.

8. Treibstoffzusammensetzung, die Mitteldestillattreibstoff mit 3 bis 1500 mg/l des Konzentrats nach einem der Ansprüche 1 bis 7 enthält.

9. Treibstoffzusammensetzung umfassend einen Mitteldestillattreibstoff und 1 bis 1400 mg/l N,N-Dimethylcyclohexylamin, 0 bis 400 mg/l N,N-Di(ortho-hydroxyaryliden)-1,2-alkylendiamin und 1 bis 1100 mg/l einer Mannich-Base, die das Reaktionsprodukt aus einem Aldehyd, einem Amin und einem Alkylphenol ist, das ausgewählt ist aus (a) einem gehinderten Phenol mit der Formel in der R₁, R₂ und R₃ unabhängig voneinander aus Wasserstoff, t-Butyl, t-Amyl und Isopropyl ausgewählt sind, mit der Maßgabe, daß mindestens einer der Reste R₁, R₂ und R₃ Wasserstoff ist und mindestens einer der Reste R₁ und R₂ t-Butyl, t-Amyl oder Isopropyl ist, und (b) einem p-Alkylphenol mit der Formel in der R_{bis} C₃₀- Alkyl ist.

10. Treibstoffzusammensetzung nach Anspruch 9, in der das Aldehyd Formaldehyd ist und das Amin aus einer oder mehreren der folgenden Substanzen ausgewählt ist:
A. Alkylmonoamine der Formel in der R₅ aus H und C₁- bis C₅-Alkyl und R₆ aus C₁ bis C₁₄-Alkyl und der Gruppe -(CH₂)n-OR₇, in der n 1 - 10 und R₇ C₁- bis C₂₀-Alkyl ist, ausgewählt ist;
B. Alkyldiamine der Formel in der R₅ aus H und C₁- bis C₅-Alkyl ausgewählt ist, R₈ C₁- bis C₆-Alkylen ist, und A und B unabhängig voneinander aus H, C₁- bis C₅-Alkyl, monohydroxysubstitiertem C₁- bis C₅-Alkyl und der Gruppe (CH₂)n-OR₇, in der n 1 bis 10 ist und R₇ C₁-bis C₂₀-Alkyl ist, ausgewählt sind;
C. Ethylenpolyamine der Formel
H₂(̵(CH₂)₂NH)̵ₙH, in der n 2 bis 10 ist, und
D. Cyclische Amine der Formel in der n und m unabhängig voneinander ganze Zahlen von 1 bis 3 sind und X ausgewählt ist aus der Gruppe CH₂, O, S und NR₉, in der R₉ H, C₁- bis C₁₀-Alkyl ist, oder der Gruppe (CH₂)ₙ-NH₂, in der n 1 bis 10 ist.

## Revendications

1. Concentré d'additifs pour combustible, comprenant un mélange de N,N-diméthylcyclohexylamine et d'une base de Mannich qui est le produit de réaction d'un aldéhyde, d'une amine primaire ou secondaire et d'un alkylphénol choisi entre (a) un phénol à encombrement stérique répondant à la formule : dans laquelle R₁, R₂, R₃ sont choisis, indépendamment, entre l'hydrogène et les radicaux tertio-butyle, tertio-amyle et isopropyle, sous réserve que l'un au moins de R₁, R₂ et R₃ soit l'hydrogène et que l'un au moins de R₁ et R₂ soit un radical tertio-butyle, tertio-amyle ou isopropyle ; et (b) un p-alkylphénol répondant à la formule : dans laquelle R₄ est un groupe alkyle en C₉ à C₃₀ ; ledit concentré contenant, sur la base de son poids total, 25 à 95 % en poids de N,N-diméthylcyclohexylamine et 5 à 75 % en poids de base de Mannich.

2. Concentré suivant la revendication 1, qui contient aussi 1 à 25 % en poids de N,N′-di(ortho-hydroxy-arylidène)-1,2-alkylènediamine comme désactivateur des métaux.

3. Concentré suivant la revendication 1 ou 2, dans lequel l'aldéhyde est le formaldéhyde et l'amine consiste en une ou plusieurs des amines suivantes :
A. des alkylmono-amines de formule : dans laquelle R₅ est choisi entre H et des radicaux alkyle en C₁ à C₅, et R₆ est choisi entre des radicaux alkyle en C₁ à C₁₄ et le groupe -(CH₂)ₙ-OR₇ dans lequel n a une valeur de 1 à 10 et R₇ est un groupe alkyle en C₁ à C₂₀,
B. des alkyldiamines de formule : dans laquelle R₅ est choisi entre H et un groupe alkyle en C₁ à C₅, R₈ est un groupe alkylène en C₁ à C₆ et A et B sont choisis, indépendamment, entre H, un groupe alkyle en C₁ à C₅, alkyle en C₁ à C₅ portant un substituant hydroxy et le groupe (CH₂)ₙ-OR₇ dans lequel n a une valeur de 1 à 10 et R₇ est un groupe alkyle en C₁ à C₂₀,
C. des éthylènepolyamines de formule :${\text{H₂N(̵(CH₂)₂NH)̵}}_{\text{n}} \text{H}$ dans laquelle n a une valeur de 2 à 10, et
D. des amines cycliques de formule : dans laquelle n et m sont, indépendamment, des nombres entiers de 1 à 3, X est choisi entre CH₂, O, S et NR₉, où R₉ représente H, un radical alkyle en C₁ à C₁₀ ou le groupe (CH₂)ₙ-NH₂ dans lequel n a une valeur de 1 à 10.

4. Concentré suivant l'une quelconque des revendications précédentes, dans lequel le phénol est un phénol à encombrement stérique et la base de Mannich comprend des N-[3,5-di-tertio-butyl-4-hydroxybenzyl]-tertio-alkylamines à groupes tertio-alkyle mixtes en C₁₂ à C₁₄, la N,N-diméthyl-3,5-di-tertio-butyl-4-hydroxybenzylamine, un composé de formule : dans laquelle R₁ et R₂ sont choisis, indépendamment, entre l'hydrogène, les radicaux tertio-butyle, tertio-amyle et isopropyle sous réserve que l'un au moins de R₁ et R₂ soit un radical tertio-butyle, tertio-amyle ou isopropyle, ou un composé de formule : dans laquelle R₁ et R₂ sont choisis, indépendamment, entre l'hydrogène, les radicaux tertio-butyle, tertio-amyle et isopropyle, sous réserve que l'un au moins de R₁ et R₂ soit un radical tertio-butyle, tertio-amyle ou isopropyle.

5. Concentré suivant l'une quelconque des revendications 1 à 3, dans lequel le phénol est un p-alkylphénol et la base de Mannich comprend le N,N-diméthyl-N′-[2-hydroxy-5-dodécylbenzyl]-1,3-diaminopropane.

6. Concentré suivant la revendication 2, dans lequel le désactivateur de métaux est la N,N′-disalicylidène-1,2-propylènediamine et la base de Mannich est le produit de réaction du formaldéhyde, du 2,6-di-tertio-butylphénol et d'une amine choisie entre le 1,3-diaminopropane, le 1,2-diaminopropane, des tertio-alkylamines à groupes alkyle mixtes en C₁₂ à C₁₄ et la diméthylamine.

7. Concentré suivant la revendication 2, dans lequel le désactivateur de métaux est la N,N′-disalicylidène1,2-propylènediamine et la base de Mannich est le produit de réaction du formaldéhyde, du p-dodécylphénol et du N,N-diméthyl-1,3-diaminopropane.

8. Composition de combustible, comprenant un combustible à base de distillat moyen contenant 3 à 1500 mg/l du concentré suivant l'une quelconque des revendications 1 à 7.

9. Composition de combustible, comprenant un combustible à base de distillat moyen et 1 à 1400 mg/l de N,N-diméthylcyclohexylamine, 0 à 400 mg/l de N,N-di(ortho-hydroxy-arylidène)-1,2-alkylènediamine et 1 à 1100 mg/l d'une base de Mannich qui est le produit de réaction d'un aldéhyde, d'une amine et d'un alkylphénol choisi entre (a) un phénol à encombrement stérique répondant à la formule : dans laquelle R₁, R₂, R₃ sont choisis, indépendamment, entre l'hydrogène, les radicaux tertio-butyle, tertio-amyle et isopropyle, sous réserve que l'un au moins de R₁, R₂ et R₃ soit l'hydrogène et que l'un au moins de R₁ et R₂ soit un radical tertio-butyle, tertio-amyle ou isopropyle ; et (b) un p-alkylphénol répondant à la formule : dans laquelle R₄ est un radical alkyle en C₉ à C₃₀.

10. Composition de combustible suivant la revendication 9, dans laquelle l'aldéhyde est le formaldéhyde et l'amine est une ou plusieurs des amines suivantes :
A. des alkylmono-amines de formule : où R₅ est choisi entre H et un radical alkyle en C₁ à C₅, et R₆ est choisi entre un radical alkyle en C₁ à C₁₄ et le groupe -(CH₂)ₙ-OR₇ dans lequel n a une valeur de 1 à 10 et R₇ est un radical alkyle en C₁ à C₂₀,
B. des alkyldiamines de formule : dans laquelle R₅ est choisi entre H et un radical alkyle en C₁ à C₅, R₈ est un radical alkylène en C₁ à C₆ et A et B sont choisis, indépendamment, entre H, un radical alkyle en C₁ à C₅, alkyle en C₁ à C₅ portant un substituant hydroxy et le groupe (CH₂)ₙ-OR₇ dans lequel n a une valeur de 1 à 10 et R₇ est un radical alkyle en C₁ à C₂₀,
C. des éthylènepolyamines de formule :${\text{H₂N(̵(CH₂)₂NH)̵}}_{\text{n}} \text{H}$ dans laquelle n a une valeur de 2 à 10, et
D. des amines cycliques de formule : dans laquelle n et m représentent, indépendamment, des nombres entiers de 1 à 3, X est choisi entre CH₂, O, S et un groupe NR₉ dans lequel R₉ représente H, un radical alkyle en C₁ à C₁₀ ou le groupe (CH₂)ₙ-NH₂ dans lequel n a une valeur de 1 à 10.
